

## UNITED STATES PATENT OFFICE

2,604,397

## CHEMICAL SENSITIZATION OF PHOTOGRAPHIC EMULSIONS

Wesley G. Lowe and Jean E. Jones, Rochester, N. Y., assignors to Eastman Kodak Company, Rochester, N. Y., a corporation of New Jersey

No Drawing. Application November 18, 1948,  
Serial No. 60,816

11 Claims. (Cl. 95—7)

## 1

This invention relates to photographic emulsions and more particularly to chemical sensitizers therefor.

It is well known that silver halide emulsions may be chemically sensitized with a variety of materials so as to increase the speed and generally the gamma of the emulsion as opposed to optical sensitization in which the optical range of sensitivity is increased. Depending upon the materials and methods employed, it is generally regarded that chemical sensitization results in either the formation of silver sulfide on the surface of the silver halide crystal thus increasing sensitivity or the formation of small amounts of silver from the reduction of silver halide. The present invention is concerned with chemical sensitization apparently of the latter type.

We have discovered that when photographic silver halide emulsions are chemically sensitized with water-soluble salts furnishing the sulfoxalate ion, appreciable increases in light sensitivity are obtained. Therefore, one object of our invention is to provide novel chemically sensitized emulsions. Another object is to provide silver halide emulsions containing sulfoxalate sensitizing as well as sensitivity due to other chemical and optical sensitizers. Other objects will appear from the following description of our invention.

The objects of our invention are accomplished by incorporating into photographic emulsions a water-soluble formaldehyde sulfoxalate salt such as an alkali metal formaldehyde sulfoxalate, particularly sodium formaldehyde sulfoxalate. The novel sensitizers are incorporated in the emulsions at any stage in their preparation but preferably before digestion is complete. Generally in order to obtain the optimum sensitizing effect we heat the emulsion after addition of the sulfoxalate sensitizer. The sensitizers may be used in conjunction with other chemical and optical sensitizers such as the well known sulfur sensitizing compounds; for example, those disclosed in Sheppard U. S. Patents 1,574,944 granted March 2, 1926, and 1,623,499, granted April 5, 1927, and may be employed before, after or simultaneously with such sulfur sensitizing and in conjunction with sensitizing dyes. Also our novel sensitizers are useful with a variety of emulsions producing pronounced speed increases in either negative or positive types of emulsions.

Our invention will now be illustrated by reference to the following specific examples:

## 2

## Example 1

100 cc. of a bromo-iodide positive type of emulsion containing silver halide obtained from 20 grams of silver nitrate and peptized with a gelatin derivative by the process disclosed in the pending Lowe et al. U. S. application Serial No. 768,478 filed August 13, 1947, was adjusted to a pH of 4.5, then treated at 130° F. with 3.0 mg. of sodium formaldehyde sulfoxalate and heating continued at this temperature for 20 minutes. Following this, the emulsion was cooled to 100° F. and the pH raised to 6.0 with sodium hydroxide solution. To samples of the resultant emulsion was added hydrophilic colloid material such as gelatin or polyvinyl alcohol, respectively, and after addition of the usual emulsion addenda, the emulsions were coated and dried in the usual manner. After exposure in an Eastman Type 2B Sensitometer (J. Soc. Mot. Pict. Eng. 17 (1931) p. 536) and processing in a developer solution of the following composition for six minutes, the emulsions were found to have materially increased in speed, as shown in the table following (samples B and F compared to samples A and E).

|                             | Developer |      |
|-----------------------------|-----------|------|
| Water                       | liter     | 1    |
| p-Methylaminophenol sulfate | grams     | 0.3  |
| Hydroquinone                | do        | 6.0  |
| Sodium Sulfite (dry)        | do        | 38.0 |
| Sodium bisulfite            | do        | 1.2  |
| Sodium carbonate (dry)      | do        | 19.0 |
| Potassium bromide           | do        | 0.9  |
| Citric acid                 | do        | 0.7  |

## Example 2

100 cc. of the same type of emulsion as was used in Example 1 but which had previously been sensitized with a sulfur type of sensitizer e. g. allyl thiourea, as described in the Lowe et al. invention, was adjusted to pH 4.5 by dilute acetic acid and treated with sodium formaldehyde sulfoxalate as in Example 1 and samples combined with gelatin and polyvinyl alcohol, respectively, to obtain emulsions the sensitivities of which are distinctly higher than obtained by using either sensitizer separately as is shown in the table following (samples D and H compared to samples B, C, F and G).

## Example 3

100 cc. of emulsion prepared as described in Example 2 (sensitized with sulfur and sulfoxalate sensitizers) were precipitated with dilute sulfuric acid and washed twice with distilled water. After

repeptizing the grains, the pH was adjusted to 6.0, the emulsion heated to 120° F. and 1.0 mg. of potassium auric chloride was added. After five minutes the temperature was lowered to 100° F., the emulsion was added to gelatin and coated and dried as usual. The characteristics of this emulsion having combined sulfur, sulfoxalate and gold sensitizing, are shown in the table (sample K compared to samples I, J and L).

| Sample | Chemical Sensitizer             | Vehicle           | Gamma | Fog | 10/E Speed<br>at dens. =<br>0.2 above<br>fog |
|--------|---------------------------------|-------------------|-------|-----|----------------------------------------------|
| A      | None                            | Gelatin           | .76   | .02 | .39                                          |
| B      | Sulfoxalate                     | do                | 1.58  | .02 | .80                                          |
| C      | Sulfur type                     | do                | 2.84  | .03 | 5.0                                          |
| D      | Sulfur and Sulfoxalate          | do                | 3.10  | .07 | 9.0                                          |
| E      | None                            | Polyvinyl Alcohol | .72   | .02 | .35                                          |
| F      | Sulfoxalate                     | do                | 1.13  | .02 | .45                                          |
| G      | Sulfur type                     | do                | 2.52  | .03 | 3.55                                         |
| H      | Sulfur and Sulfoxalate          | do                | 2.51  | .05 | 4.70                                         |
| I      | Sulfur type                     | Gelatin           | 2.6   | .02 | 4.3                                          |
| J      | Sulfur and Sulfoxalate          | do                | 3.1   | .07 | 7.3                                          |
| K      | Sulfur and Sulfoxalate and Gold | do                | 3.2   | .09 | 14.0                                         |
| L      | Sulfur and Gold                 | do                | 3.5   | .04 | 6.5                                          |

It is apparent from the above data that the new sulfoxalate sensitizer used in conjunction with a sulphur sensitizer has effected a speed increase greater than that expected from the activity of the individual sensitizers when used alone. However, the speed increases obtained in absence of sulfur sensitizing are appreciable and valuable.

In the manner of the above examples, other types of silver halide emulsions may be treated with our novel sensitizers alone or in conjunction with other chemical or optical sensitizers. The amount of the sulfoxalate sensitizer incorporated into an emulsion may, depending upon the type of emulsion used, vary somewhat from the optimum amount employed in the above examples, one-fifth to five times as much sensitizer producing emulsion of useful sensitivity that is, from about 0.03 to 0.75 gram of the sensitizer per kilogram of silver nitrate used in making the emulsion and converted to silver halide. Less heating is usually required when the larger amounts are employed and conversely, when using the smaller quantities of sensitizer.

The novel sensitizers may, in general, be employed in emulsions containing hydrophilic colloid vehicles; for example, gelatin, polyvinyl alcohol, partially hydrolyzed cellulose esters and co-polymers of polyvinyl alcohol. The ratio of colloid to silver halide present during digestion is not critical in this type of sensitizing since the digestion conditions can be readily adjusted as is well known in the art of sulfur sensitizing. The sensitizers are suitable for the well known types of silver chloride, silver bromide and silver iodide emulsions and emulsions containing mixtures of these halides. Also the emulsions may contain the usual addenda including antifoggants, spreading agents, coupler compounds, etc. Such emulsions are adaptable to use in forming single as well as multi-layer films useful in color photography which customarily include two or more emulsion layers on a support sensitized to different regions of the visible spectrum and may or may not contain coupler compounds. According to our invention such color films carry at least one emulsion layer containing a sulfoxalate salt sensitizing agent.

Our invention having been described, we would have it understood that the preceding description is by way of example only and that our inven-

tion is to be taken as limited only by the scope of the appended claims.

What we claim is:

5 1. A light-sensitive photographic emulsion comprising silver halide and from about 0.03 to 0.75 gram per kilogram of silver nitrate used in making the emulsion and converted to silver halide, of a water-soluble formaldehyde sulfoxalate salt as a sensitizing agent.

2. A light-sensitive photographic emulsion comprising silver halide and from about 0.03 to 0.75 gram per kilogram of silver nitrate used in making the emulsion and converted to silver halide, of sodium formaldehyde sulfoxalate as a sensitizing agent.

30 3. A light-sensitive photographic emulsion comprising sulfur sensitized silver halide and from about 0.03 to 0.75 gram per kilogram of silver nitrate used in making the emulsion and converted to silver halide, of sodium formaldehyde sulfoxalate as an additional sensitizing agent.

35 4. A light-sensitive photographic emulsion comprising silver halide sensitized with a sulfur sensitizing compound, a gold salt sensitizer and sodium formaldehyde sulfoxalate.

40 5. A light-sensitive photographic emulsion comprising silver halide uniformly dispersed in a hydrophilic colloid vehicle and sensitized with from about 0.03 to 0.75 gram per kilogram of silver nitrate used in making the emulsion and converted to silver halide, of a water-soluble formaldehyde sulfoxalate salt.

50 6. A light-sensitive photographic emulsion comprising silver halide uniformly dispersed in gelatin and sensitized with from about 0.03 to 0.75 gram per kilogram of silver nitrate used in making the emulsion and converted to silver halide, of sodium formaldehyde sulfoxalate.

55 7. A light-sensitive photographic emulsion comprising silver halide uniformly dispersed in polyvinyl alcohol and sensitized with from about 0.03 to 0.75 gram per kilogram of silver nitrate used in making the emulsion and converted to silver halide, of sodium formaldehyde sulfoxalate.

60 8. The method of increasing the speed of a photographic silver halide emulsion which comprises imparting sulfur sensitivity to said emulsion, adjusting the pH of said emulsion to below neutrality, and effecting a further increase in sensitivity by digesting said emulsion in the presence of a water-soluble formaldehyde sulfoxalate salt.

65 9. The method of increasing the speed of a photographic silver halide emulsion which comprises imparting sulfur sensitivity to said emulsion, adjusting the pH of said emulsion to below neutrality and effecting a further increase in

sensitivity by digesting said emulsion in the presence of sodium formaldehyde sulfoxalate.

10. The method of sensitizing a photographic silver halide emulsion which comprises digesting said emulsion in the presence of a sulfur sensitizing agent and a water-soluble formaldehyde sulfoxalate salt.

11. The method of sensitizing a photographic silver halide emulsion which comprises digesting said emulsion in the presence of a sulfur sensitizing agent and sodium formaldehyde sulfoxalate.

WESLEY G. LOWE.  
JEAN E. JONES.

## REFERENCES CITED

The following references are of record in the file of this patent:

## UNITED STATES PATENTS

| Number    | Name            | Date          |
|-----------|-----------------|---------------|
| 1,763,533 | Miller          | June 10, 1930 |
| 2,059,817 | Sheppard et al. | Nov. 3, 1936  |

## FOREIGN PATENTS

| Number  | Country       | Date          |
|---------|---------------|---------------|
| 496,049 | Great Britain | Nov. 21, 1938 |